

## 1

3,272,635

### COMPOSITIONS CONTAINING LEUCO XANTHENE DYES AND SUITABLE ACTIVATORS

Robert H. Sprague, Chagrin Falls, John A. Stewart, Parma, and James M. Lewis, Cleveland, Ohio, assignors to Horizons Incorporated, Cleveland, Ohio, a corporation of New Jersey  
 No Drawing. Filed Apr. 17, 1963, Ser. No. 273,569  
 7 Claims. (Cl. 96—90)

This invention relates to non-silver photosensitive compositions which print-out an image directly upon exposure to a suitable dosage of visible light, and to the use to such compositions as thin films in photographic processes. More particularly this invention relates to photosensitive compositions comprising at least one colorless leuco compound which when intimately admixed with one or more colorless activator compounds, yields a mixture which when exposed to visible light prints out a visible image directly, at speeds which are of practical significance, and to the processing of such compositions to yield a permanent useful image.

#### (1) THE LEUCO COMPOUNDS

The leuco compounds which may be utilized in accordance with the present invention comprise two recognized classes of dye forming colorless compounds which are generally similar to the leuco triarylmethane dyes except that they are characterized by the presence of one or more bridging hetero atoms and therefore are compounds which may be represented by the general formulas



and



wherein each R is selected from the group consisting of H, lower alkyl and aryl and may be the same or different and R<sub>3</sub> is selected from the group consisting of H, alkyl and aryl, including particularly



and wherein Z represents a member selected from the group consisting of >O, >S, >Se and >NH.

As indicated, the preferred leuco compounds of this class are substituted in the 3,6-positions and include 3,6-bis(dimethylamino)-9-(p-dimethylaminophenyl)-xanthene and 3,6-bis(diethylamino)-9-(p-dimethylaminophenyl)-xanthene.

## 2

3,6-bis(diethylamino)-9-(p-diethylaminophenyl)-xanthene

3,6-bis(dimethylamino)-9-(p-dimethylaminophenyl)-thioxanthene

#### (2) THE ACTIVATORS

A diverse group of colorless >C=O containing organic compounds have been found to be useful in the present invention. These compounds may be grouped as follows:

10 (1) Carboxylic acids represented by the general formula



15 wherein R' stands for either aryl or alkaryl;

(2) Acyclic keto compounds of the general formula



20 wherein A represents alkyl, alkaryl or aryl, and R'' is selected from the group consisting of aryl,



25 and



30 wherein R<sub>a</sub> is selected from the group consisting of H, alkyl, aralkyl, aryl, and



35 R<sub>b</sub> being selected from the group consisting of H, alkyl, aralkyl and aryl;

(3) Cyclic keto compounds represented by the general formula



40 where Q represents the non-metallic atoms necessary to complete a five- or six-membered heterocyclic ring and 45 wherein the keto oxygen is attached to a ring carbon in said ring.

#### (3) EVALUATION PROCEDURE

The data reported in the tables which follow is the 50 result of tests establishing the effect of visible light on mixtures of various activator compounds with the indicated leuco bases. In general one of three procedures was followed.

In the first two, a mixture is prepared consisting of 55 equal parts by volume of acetone and a 10% solution of polystyrene in benzene, 2 cc. of each being used in most instances. Then the indicated weights of the leuco compound and of the activator were dissolved in the mixture. The resulting composition formed from origi-

60 nally colorless materials had a cloudy or hazy appearance or a faint pinkish color in most instances. The composition was coated by means of a Bird applicator on 500-D Mylar in a coating having an 0.0015 inch wet thickness and the coating was permitted to dry in air.

65 Thereafter the composition was exposed either to a photo-flood lamp through a step tablet or on an Eastman Kodak sensitometer with a suitable filter.

When the composition was exposed to a General Electric 500 watt RFL 2 Photoflood lamp exposures were through a #2 silver step wedge for a 5 minute interval at a distance of 12 inches from lamp to test materials. The density and number of steps visible in the image were read, after fixing the image by solvent wash or by heat.

When the composition was exposed on an Eastman Kodak No. 101 sensitometer the light was converted by the use of a 78AA filter, to equal mean noon-day light. The resulting image was fixed by a solvent wash or by exposure to heat. Thereafter the density of the image was read and the L.E.S. was computed as described below.

In a third procedure, the polystyrene was omitted from the compositions and instead a mixture of benzene and acetone was used as the solvent for the indicated amounts of the leuco compound and the activator. The solution was poured onto filter paper and the photo-sensitive material was then exposed through an Eastman No. 2 Step Tablet to one General Electric Reflector Photoflood lamp for 30 seconds at a distance of 12 inches from the lamp to the sensitive material. The densities of the resulting step wedge were read on an Eastman No. 1 color densitometer through the green filter.

L.E.S. (abbreviation for light exposure speed) refers to a speed rating system developed at the Wright Air Development Division of Air Research and Development Command (USAF), and is defined as the reciprocal of

the exposure in meter candle seconds which is required to produce a double diffuse reflection density of 0.2 density units above base plus fog. As in the more conventional ASA system used to rate silver halide films, the higher the L.E.S. number the faster the film is.

Compositions consisting of the indicated weight of 3,6-bis-(dimethylamino)-9-(p-dimethylaminophenyl)xanthene (hereinafter identified as D-179), and the indicated weight of the specified activator dissolved in a mixture of acetone and 2 cc. of a 10% solution of polystyrene in benzene coated 0.0015-inch wet thickness on Mylar and air-dried were exposed using an Eastman No. 101 sensitometer for the indicated time with the light converted by the use of a 78AA Eastman filter to equal mean noonday light or to one General Electric No. 2 Reflector Photoflood lamp (RFL2), at a distance of 12 inches. An Eastman Kodak No. 2 Step Tablet was used to print a step tablet. The exposed material was stabilized by two or more successive rinses in a mixture of 1 part acetone and 4 parts petroleum ether, or by being maintained at 125° C. in a convection-type oven for four (4) minutes. The stabilized material was reexposed for 5 minutes to the RFL2 with no darkening. The densities in the resulting step wedge were read with an Eastman No. 1 color densitometer using the green filter, the results for the photoflood exposures are reported in Table I and the densitometer exposures in Table II.

Table I

| No.     | Activators Used With D-179                                   | Weight, mg. | Type of Fixing | Exp. Min. | No. of Steps | Densities, RFL2 |            |      |
|---------|--------------------------------------------------------------|-------------|----------------|-----------|--------------|-----------------|------------|------|
|         |                                                              |             |                |           |              | Gross           | Base + Fog | Net  |
| 1.....  | Benzoic Acid.....                                            | 50          | Heat.....      | 5         | 19           | 1.55            | 0.36       | 1.19 |
|         | D-179.....                                                   | 50          | Solvent.....   | 5         | 21           | 1.57            | 0.25       | 1.32 |
| 2.....  | $\alpha$ -Naphthoic Acid.....                                | 50          | Heat.....      | 5         | 21           | 2.57            | 0.33       | 2.24 |
|         | D-179.....                                                   | 50          | Solvent.....   | 5         | 21           | 2.12            | 0.25       | 1.87 |
| 3.....  | 1-Hydroxy-2-naphthoic Acid.....                              | 50          | .....do.....   | 5         | 21           | 2.46            | 0.15       | 2.31 |
|         | D-179.....                                                   | 50          | .....do.....   | 5         | 21           | 2.02            | 0.23       | 1.79 |
| 4.....  | 3-Hydroxy-2-naphthoic Acid.....                              | 50          | Heat.....      | 5         | 18           | 1.85            | 0.34       | 1.51 |
|         | D-179.....                                                   | 50          | Solvent.....   | 5         | 21           | 1.45            | 0.25       | 1.20 |
| 5.....  | 2-Mercaptobenzoic Acid (thiosalicylic Acid).....             | 50          | Solvent.....   | 5         | 21           | 2.00            | 0.15       | 1.85 |
|         | D-179.....                                                   | 50          | Solvent.....   | 5         | 21           | 2.60            | 0.29       | 2.31 |
| 6.....  | Phenyl Acetic Acid.....                                      | 50          | .....do.....   | 5         | 21           | 2.22            | 0.13       | 2.09 |
|         | D-179.....                                                   | 50          | .....do.....   | 5         | 21           | 2.22            | 0.13       | 2.09 |
| 7.....  | 1-Naphthylacetic Acid.....                                   | 50          | Heat.....      | 5         | 8            | 0.48            | 0.28       | 0.20 |
|         | D-179.....                                                   | 50          | .....do.....   | 5         | 11           | 0.72            | 0.28       | 0.44 |
| 8.....  | 2,4-Dichlorophenoxyacetic Acid.....                          | 50          | .....do.....   | 5         | 11           | 1.30            | 0.28       | 1.02 |
|         | D-179.....                                                   | 50          | .....do.....   | 5         | 11           | 1.77            | 0.78       | 0.99 |
| 9.....  | 2-Mercapto-1-naphthylacetic Acid.....                        | 50          | Solvent.....   | 5         | 21           | 1.31            | 0.30       | 1.01 |
|         | D-179.....                                                   | 50          | Heat.....      | 5         | 12           | 0.87            | 0.28       | 0.59 |
| 10..... | Tribromonacetophenone.....                                   | 50          | .....do.....   | 5         | 12           | 1.61            | 0.20       | 1.41 |
|         | D-179.....                                                   | 100         | .....do.....   | 5         | 10           | 1.19            | 0.32       | 0.87 |
| 11..... | p-Nitroacetanilide.....                                      | 100         | Heat.....      | 5         | 6            | 0.77            | 0.48       | 0.29 |
|         | D-179.....                                                   | 50          | Solvent.....   | 5         | 9            | 0.60            | 0.16       | 0.44 |
| 12..... | p-Phenylacetanilide.....                                     | 100         | .....do.....   | 5         | 17           | 1.77            | 0.24       | 1.53 |
|         | D-179.....                                                   | 50          | .....do.....   | 5         | 14           | 2.17            | 0.20       | 1.97 |
| 13..... | ( $\alpha$ , $\alpha$ , $\alpha$ -Trichloroacetanilide)..... | 100         | Heat.....      | 5         | 11           | 2.25            | 0.35       | 1.90 |
|         | D-179.....                                                   | 50          | Solvent.....   | 5         | 13           | 1.49            | 0.13       | 1.36 |
| 14..... | 1-Aceto-2-naphthol.....                                      | 15          | .....do.....   | 5         | 11           | 2.20            | 0.17       | 2.03 |
|         | D-179.....                                                   | 50          | .....do.....   | 5         | 13           | 0.95            | 0.35       | 0.60 |
| 15..... | (Acetoacetyl)anilide.....                                    | 100         | Heat.....      | 5         | 18           | 2.36            | 0.18       | 2.18 |
|         | D-179.....                                                   | 50          | .....do.....   | 5         | 12           | 1.16            | 0.44       | 0.72 |
| 16..... | (Acetoacet-2,5-dichloroanilide).....                         | 100         | Heat.....      | 5         | 17           | 1.77            | 0.24       | 1.53 |
|         | D-179.....                                                   | 50          | .....do.....   | 5         | 14           | 2.17            | 0.20       | 1.97 |
| 17..... | (Acetoacet-2,5-dichloroanilide).....                         | 100         | Heat.....      | 5         | 11           | 2.25            | 0.35       | 1.90 |
|         | D-179.....                                                   | 50          | Solvent.....   | 5         | 13           | 1.49            | 0.13       | 1.36 |
| 18..... | Acetoacet-2,5-dichloro-N-benzoylanilide.....                 | 100         | Heat.....      | 5         | 6            | 0.77            | 0.48       | 0.29 |
|         | D-179.....                                                   | 100         | Solvent.....   | 5         | 9            | 0.60            | 0.16       | 0.44 |
| 19..... | (Acetoacet-2,5-dichloro-N-(m-nitrobenzoyl)anilide).....      | 100         | .....do.....   | 5         | 12           | 1.16            | 0.44       | 0.72 |
|         | D-179.....                                                   | 50          | .....do.....   | 5         | 13           | 0.95            | 0.35       | 0.60 |
| 20..... | (Acetoacet-2,5-dichloro-N-butyrylanilide).....               | 100         | Heat.....      | 5         | 18           | 2.36            | 0.18       | 2.18 |
|         | D-179.....                                                   | 50          | .....do.....   | 5         | 12           | 1.16            | 0.44       | 0.72 |
| 21..... | Mono-Benzoyl Aceto-4,3',3'-dichlorobenzidide.....            | 100         | .....do.....   | 5         | 12           | 1.16            | 0.44       | 0.72 |
|         | D-179.....                                                   | 50          | .....do.....   | 5         | 13           | 0.95            | 0.35       | 0.60 |
| 22..... | (Mono-Benzoylacetbenzidide).....                             | 50          | .....do.....   | 5         | 17           | 1.77            | 0.24       | 1.53 |
|         | D-179.....                                                   | 50          | .....do.....   | 5         | 14           | 2.17            | 0.20       | 1.97 |
| 23..... | (Acetoacet-2-chloro-N-butyrylanilide).....                   | 100         | Heat.....      | 5         | 11           | 2.20            | 0.17       | 2.03 |
|         | D-179.....                                                   | 50          | .....do.....   | 5         | 12           | 0.95            | 0.35       | 0.60 |
| 24..... | $\beta$ -Naphthoylacetanilide.....                           | 50          | Heat.....      | 5         | 11           | 2.25            | 0.35       | 1.90 |
|         | D-179.....                                                   | 50          | Solvent.....   | 5         | 13           | 1.49            | 0.13       | 1.36 |
| 25..... | (Phenylisoxazolone).....                                     | 100         | Heat.....      | 5         | 11           | 2.20            | 0.17       | 2.03 |
|         | D-179.....                                                   | 50          | .....do.....   | 5         | 14           | 2.17            | 0.20       | 1.97 |
| 26..... | (3-Methyl-1-phenyl-5-pyrazolone).....                        | 50          | .....do.....   | 5         | 11           | 0.55            | 0.07       | 0.48 |
|         | D-179.....                                                   | 50          | Solvent.....   | 5         | 12           | 2.32            | 0.45       | 1.87 |
| 27..... | 1,3-Diphenyl-5-pyrazolone.....                               | 50          | .....do.....   | 5         | 11           | 0.55            | 0.07       | 0.48 |
|         | D-179.....                                                   | 100         | Heat.....      | 5         | 12           | 2.32            | 0.45       | 1.87 |
| 28..... | Benzothiazolone.....                                         | 100         | .....do.....   | 5         | 12           | 2.32            | 0.45       | 1.87 |

5  
Table II

| Composition Number | Exposed, min. | No. Steps | Densities No. 101 Sensitometer |            | L.E.S.               | 5  |
|--------------------|---------------|-----------|--------------------------------|------------|----------------------|----|
|                    |               |           | Gross                          | Base + Fog |                      |    |
| 1                  | 30            | 9         | 0.56                           | 0.26       | $3.8 \times 10^{-6}$ |    |
| 2                  | 30            | 14        | 0.62                           | 0.25       | $7.6 \times 10^{-6}$ |    |
| 3                  | 30            | 10        | 1.15                           | 0.40       | $1.7 \times 10^{-5}$ |    |
| 4                  | 30            | 14        | 0.63                           | 0.11       | $1.6 \times 10^{-6}$ |    |
| 5                  | 30            | 12        | 0.52                           | 0.08       | $1.3 \times 10^{-5}$ |    |
| 6                  | 10            | 15        | 0.90                           | 0.16       | $1 \times 10^{-4}$   |    |
| 6                  | 60            | 11        | 1.31                           | 0.51       | $3.2 \times 10^{-5}$ |    |
|                    | 60            | 12        | 0.74                           | 0.22       | $5.3 \times 10^{-6}$ |    |
| 7                  | 30            | 11        | 0.65                           | 0.11       | $8.9 \times 10^{-6}$ |    |
| 8                  | 60            | 15        | 1.64                           | 0.24       | $4.7 \times 10^{-5}$ |    |
| 9                  | 30            | 12        | 0.91                           | 0.11       | $1.6 \times 10^{-5}$ |    |
| 10                 | 30            | 15        | 0.91                           | 0.20       | $2.1 \times 10^{-5}$ |    |
| 11-15              |               |           |                                |            |                      |    |
| 16                 | 30            | 9         | 0.50                           | 0.16       | $4.8 \times 10^{-6}$ |    |
| 17-24              |               |           |                                |            |                      |    |
| 25                 | 120           | 9         | 0.76                           | 0.25       | $1.6 \times 10^{-6}$ |    |
| 26                 | 30            | 14        | 0.55                           | 0.18       | $5.2 \times 10^{-6}$ |    |
| 27                 | 30            | 11        | 0.72                           | 0.05       | $2.1 \times 10^{-5}$ |    |
| 28                 | 60            | 9         | 0.76                           | 0.28       | $3.8 \times 10^{-6}$ |    |
|                    |               |           |                                |            |                      | 20 |

## FIXING

Two distinct methods of fixing or stabilizing the colored image produced have been described. In the one the exposed material is subjected to two or more 15 second rinses with a suitable solvent and in the other the exposed material is subjected to mild heat (125°) for about 4 minutes. The method of stabilization selected in any specific instance will depend to some extent upon the materials being used and it is to be noted that many of the "slower" compositions may be preferable to some of the "faster" compositions because some of the latter are less susceptible to heat or dry fixing than some of the former.

While not wishing to be bound by any specific theory as to the manner in which the exposure to visible light to an intimate mixture comprising two or more originally colorless compounds produced a colored image, it is believed that the final colored image which forms in the light struck areas is always the dye which forms as a result of oxidation of the leuco base. Furthermore it appears that when the photosensitive mixture is prepared, on mixing the compounds which are colorless, a weakly tinted mixture is formed.

It is also considered possible that the real active ingredient in the mixture is that very minute amount of an oxidized product which results when the leuco base is exposed to oxygen e.g. in the ordinary atmosphere.

Whatever the true mechanism each of the activators listed above, or mixtures of the same, bring about oxidation of the leuco compound upon exposure to a suitable dose of visible light and as a result form a direct visible print-out image in the light struck areas.

## PROPORTIONS

The relative proportions of the leuco dye bases and the activators for the same may be varied considerably from the weight proportions given by way of illustration in the examples and are preferably within the range between 10 to 1 and 1 to 10 parts by weight.

As with other photosensitive compositions if not used at the time they are prepared the compositions of the present invention would be stored in cool dark relatively dry surroundings.

Having now described the invention in accordance with the patent statutes it is not intended that it be limited except as may be required by the appended claims.

We claim:

1. A composition which prints out a visible image directly as a result of exposure to visible light said composition comprising an intimate mixture consisting essentially of

6  
(1) at least one leuco compound selected from the group consisting of leuco compounds represented by one of the following general formulas



wherein each R is selected from the group consisting of H, lower alkyl and aryl and not all of the R's need be the same and wherein R<sub>2</sub> is selected from the group consisting of H, lower alkyl and aryl and Z is selected from O, S, Se and —NH:



and wherein each R has the same meaning as indicated above and Z represents a member selected from the group consisting of O, S, Se and —NH; and

(2) at least one colorless non-toxic >C=O containing organic compound selected from the group consisting of

- (a) carboxylic acids represented by the general formula R'COOH wherein R' is selected from the group consisting of aryl and alkaryl  
(b) acyclic keto compounds represented by the general formula



wherein R'' is selected from the group consisting of aryl,



and



wherein R<sub>a</sub> is selected from the group consisting of H, alkyl, aralkyl, aryl and



R<sub>b</sub> being selected from the group consisting of H, alkyl, aralkyl and aryl; and A is selected from the group consisting of alkyl, alkaryl and aryl and

- (c) cyclic keto compounds represented by the general formula



wherein Q represents the non-metallic atoms necessary to complete a heterocyclic ring with at least 5 and not more than 6 atoms in the ring and wherein the keto oxygen is attached to a ring carbon atom is said ring;

said compounds being present in the mixture in proportions ranging between 1:10 and 10:1 relative to each other, by weight.

2. The composition of claim 1 wherein the leuco compound is a xanthene.

3. The composition of claim 2 wherein the leuco compound is a 3,6 - bis(dialkylamino) - 9 - (p - dialkylamino-phenyl)xanthene.

4. A dry film consisting of the composition of claim 1 dispersed in a thin layer on an inert support.

5. The film of claim 4 wherein the support is a film forming plastic.

6. The film of claim 4 wherein the mixture is supported by a cellulose compound selected from the group consisting of cellulose and film forming cellulose derivatives.

7. The film of claim 4 wherein the support is transparent.

## References Cited by the Examiner

## UNITED STATES PATENTS

|   |           |        |                |       |         |
|---|-----------|--------|----------------|-------|---------|
| 5 | 2,441,561 | 5/1948 | Chalkley       | ----- | 96-90 X |
|   | 2,895,892 | 7/1959 | Chalkley       | ----- | 96-90 X |
|   | 2,981,622 | 4/1961 | Chalkley       | ----- | 96-90 X |
|   | 3,121,632 | 2/1964 | Sprague et al. | ----- | 96-90 X |

NORMAN G. TORCHIN, *Primary Examiner.*

10 D. D. PRICE, *Assistant Examiner.*